

## UNITED STATES PATENT OFFICE

2,172,382

## LUBRICATING OIL

Alfred Henriksen and Bert H. Lincoln, Ponca City, Okla., assignors, by mesne assignments, to The Lubri-Zol Development Corporation, Cleveland, Ohio, a corporation of Delaware

No Drawing. Application January 26, 1933,  
Serial No. 653,667

5 Claims. (Cl. 87-9)

Our invention relates to an improved lubricating oil and more particularly to a lubricating oil having a low cold test and a high film strength.

In the production of high grade lubricating oils for present day motor equipment certain characteristics must be obtained in the finished lubricant other than viscosity, flash point, freedom from grit and other abrasive substances which were previously the controlling factors. Present day high grade lubricants must have, in addition to the above low cold test or solidification points, high film strength and increased oiliness or uncrossed.

Low cold test or solidification point of a lubricant is obtainable in the present day art by the very costly dewaxing processes. In addition to the very high cost of original equipment for dewaxing and the continued high cost of operation of dewaxing equipment, there is another objection to this method of obtaining low cold test due to certain objectionable changes in the nature of the lubricant as a direct result of the removal of the wax.

Another method of lowering the cold test of a lubricant has been described in United States Letters Patent 1,815,022 granted July 14, 1931, to Garland H. B. Davis.

In the Davis invention, a synthetic hydrocarbon oil is formed by condensing a wax hydrocarbon material with an aromatic hydrocarbon or by condensing a halogenated paraffin with an aromatic hydrocarbon. This synthetic oil when added to a lubricating oil containing a solid wax component will reduce the pour point thereof. The film strength of the lubricant, however, is decreased or at any rate not materially improved.

One object of our invention is to provide a lubricant having a lowered cold test and an increased film strength.

Other objects of our invention will appear from the following description.

In general, our method consists of halogenation of paraffin wax and the like, then reacting the halogenated wax with aromatic hydrocarbons by the reaction known as "Friedel Crafts Reaction" in order to produce a condensation product of paraffin wax and aromatic compounds. The thus prepared hydrocarbon condensation product is then halogenated. Naphthalene, anthracene and products rich in aromatic hydrocarbons and the like may be used to react with the halogenated long chain hydrocarbon. The purified, and halogenated condensation product is added to lubricants in small amounts or is added to lubricants in a blend with small amounts of halogenated fatty acids.

For example, wax is chlorinated by direct chlorination until it contains about the calculated amount of halogen for a mono-halogen product.

This will vary rather widely with the approxi-

mate average molecular weight of the wax being halogenated and may range from 10% or less of chlorine on up to 20% or more. The temperature is controlled during the halogenation step to avoid temperatures much above 300° F. Aromatic hydrocarbons such as naphthalene or anthracene are then mixed with approximately an equal weight of aluminum chloride and the chlorinated oil added slowly, while maintaining a temperature not to exceed about 160° F. An inert solvent may be used for the reacting mixture which should be constantly agitated until the reaction is completed, which is apparent from the lack of formation of large volumes of hydrogen chloride gas when fresh chlorinated wax is added. This also controls the proportions in which the chlorinated wax is added. When the reaction is apparently complete, it is desirable to increase the temperature of the reacting mixture to expel any remaining hydrogen chloride. The mass is allowed to stand until the aluminous sludge settles out or the sludge may be removed by mechanical means such as filtration. The reaction product is then placed in distilling equipment and the solvent and unreacted wax removed with as little heat as possible and under a high vacuum preferably. The recovered condensation product is a liquid hydrocarbon mixture containing slight traces of halogen, usually less than 0.4%.

The above condensation product may then be treated with halogen. To treat with halogen it is necessary only to pass the halogen through the condensation product at a temperature of about 200° F. until the proper amount of halogen has been added which may be 5% or less, 10%, 15%, 20% of the original weight of condensation product, or more. After halogenation the product may be treated with lime or clay to remove any free halogen or halogen acid and then filtered. Various solvents may be used to extract the halogenated product or it may be purified by low vacuum distillation.

As an example of the cold test lowering of the above products, a sample of high quality 350 viscosity steam refined stock with a 22° F. cold test was blended with the halogenated condensation product with the following results:

|                                                                                   | Cold test. ° F. |
|-----------------------------------------------------------------------------------|-----------------|
| Original 350 vis. lubricant                                                       | 22              |
| 99.5% original lubricant plus 0.5% condensation product treated with 5% chlorine  | 50              |
| 99.5% original lubricant plus 0.5% condensation product treated with 10% chlorine | 6               |
| 99.5% original lubricant plus 0.5% condensation product treated with 10% chlorine | 16              |

From the above table the efficiency of our product in lowering cold test is fully demonstrated. In the tests made, only 0.5% of the product of our invention was added to the lubricant, but with poorer quality lubricants and/or with higher cold test lubricants larger quantities may be used.

and may be as much as 10% or more of the volume of the original lubricant.

To prove the increased film strength of lubricants prepared according to our invention, we employ the new type Timken testing machine manufactured by the Timken Roller Bearing Company. In this machine lubricants are used between two rubbing surfaces under increasing pressure or load until the lubricant breaks down and allows metal seizure. The load required to cause seizure is a measure of the film strength of the lubricant under test. These loads converted into pounds per square inch on the rubbing surfaces gives a good comparison of the film strength of any two lubricants. In the following examples a high quality S. A. E. 40 lubricant was used and the results are reported in pound weights added to obtain film rupture and these pound weights converted into approximate pounds per square inch.

|   | Oil tested                                                                   | Pound weights | Approximate pounds per square inch |
|---|------------------------------------------------------------------------------|---------------|------------------------------------|
| 1 | Original S. A. E. 40 mineral oil                                             | 11.3          | 7,000                              |
| 2 | 99% original lubricant plus 1% of condensation product                       | 10.3          | 6,300                              |
| 3 | 99% original lubricant plus 1% condensation product treated with 6% chlorine | 17.3          | 10,500                             |

From the above it is noted that the addition of the condensation product direct to the lubricant lowers the film strength of the original lubricant. It also shows that if the condensation product is treated with chlorine the film strength of the original lubricant is greatly improved.

Small amounts of chlor stearic or other halogenated organic acids in any of the mixtures described in this invention will improve the film strength and decrease the coefficient of friction (give greater oiliness).

It will be observed that our invention begins where the Davis invention leaves off. We take the synthetic product achieved by Davis and halogenate it to increase its film strength.

Having thus described our invention, what we claim is:

1. An improved lubricating oil of relatively low pour point and comparatively high film strength comprising in combination a hydrocarbon oil and a small amount of a halogenated synthetic hydrocarbon oil obtained by halogenating, to the extent of from 5 to 20%, the condensation product obtained by the addition of a halogenated wax to a mixture of an aromatic compound and a catalyst of the type represented by aluminum chloride. 10

2. An improved lubricating oil of relatively low pour point and comparatively high film strength comprising in combination a hydrocarbon oil and a small amount of a chlorinated synthetic hydrocarbon oil obtained by chlorinating, to the extent of from 10 to 20 percent, the condensation product obtained by the addition of chlorinated wax to a mixture of an aromatic compound and a catalyst of the type represented by aluminum chloride. 15

3. An improved lubricating oil of relatively low pour point and comparatively high film strength comprising in combination a hydrocarbon oil and a small amount of a chlorinated synthetic hydrocarbon oil obtained by chlorinating, to the extent of from 5 to 20 percent, the condensation product obtained by the addition of chlorinated paraffin wax to a mixture of naphthalene and aluminum chloride. 20

4. An improved lubricating oil of relatively low pour point and comparatively high film strength comprising a blend of hydrocarbon oil and small amounts of both a halogenated fatty acid and a synthetic oil formed by halogenating the reaction product obtained by the addition of a chlorinated wax to a mixture of an aromatic compound and a catalyst of the type represented by aluminum chloride. 30

5. An improved lubricating oil of relatively low pour point and comparatively high film strength comprising a blend of hydrocarbon oil and small amounts of chlorinated stearic acid and a synthetic oil formed by halogenating the reaction product obtained by the addition of chlorinated wax to a mixture of naphthalene and aluminum chloride. 40

ALFRED HENRIKSEN.  
BERT H. LINCOLN.